

## UNITED STATES PATENT OFFICE.

HENDRIK JAN JAKOB JANSSEN, OF ARNHEM, NETHERLANDS, ASSIGNOR TO NAAM-  
LOOZE VENNOOTSCHAP NEDERLANDSCHE KUNSTZIJDEFABRIEK, OF ARNHEM,  
NETHERLANDS.

TREATMENT OF TEXTILE FIBERS, YARNS, FABRICS, OR THE LIKE FOR OBTAINING  
EFFECTS OF COLOR OR LUSTER OR BOTH.

No Drawing. Application filed May 28, 1925, Serial No. 33,508, and in the Netherlands April 7, 1925.

This invention is based on the observation that cellulose threads and yarns, whether artificial or natural, for instance artificial

silk, cotton and other textile fibers, such as or colorless metal compounds, e. g. into sulphides which are deposited firmly on or in the fibers.

5 <sup>55</sup> wool and natural silk, may be dyed differently or given a different luster, in the same dyeing-bath, or both dyed differently and given a different luster, if there is allowed to form or deposit upon or in a part of the 10 fibers a precipitate of sulphur while another part of the fibers is left unchanged. Also, fibers having different sulphur contents, together with fibers without sulphur, may be treated in this manner. This applies both

to mixtures of different fibers and to different parts of the same fiber. Such a precipitate of sulphur can be produced in various ways. For example, the fibers may be saturated with a polysulphide solution of 15 an alkaline metal or of ammonia and afterwards treated in an acid bath. Another method consists in dissolving sulphur in an organic solvent, saturating the thread with the solution and subsequently evaporating 20 the solvent, whereupon there remains in the fibers a finely subdivided precipitate of sulphur. It is also possible to use for the process unbleached viscose silk which still contains sulphur.

Obviously other metal salts having different colored sulphur compounds and capable of forming a precipitate on the fibers by means of the sulphur (for instance, silver-, nickel-, cadmium-, antimony-, tin-, or iron-salts) may be used. When the metal compound has been formed on the unbleached threads and the fabric has been 25 washed the latter may be brought into a second dye-bath containing, for instance, an organic dyestuff for which the metal compound on the sulphured fibers can act as a mordant to dye the sulphured fibers a different color from that which the dyestuff produces on the non-sulphured fibers. If the metal mordant is itself colored there is produced by the addition of the second dye- 30 stuff a mixed dyeing. For instance it is possible to convert the sulphur compound of the metal on the fibers into oxides, and to dye afterwards with dyestuffs like alizarine, which form lakes of different colors with the oxides, e. g. iron and aluminium. 35

In certain cases it is possible after the dyeing to extract the metal mordant from the sulphured fibers without interfering with the difference of color between the sulphured and non-sulphured fibers or the dyestuff itself.

The invention can be applied in many manners.

It will be obvious that the processes described above can be applied not only to the fibers but also to fabrics made therefrom, knitted or woven piece goods or the like.

Different quantities of the fibrous material may be treated with unequal quantities 40

45 of suitable metallic salt solutions into colored

50

55

60

of sulphur; or the sulphured fibers, or a part of them, may be desulphured to different degrees, so that 10, 20 or more per cent of the original sulphur may remain, which may be attained by the use of mild agents for dissolving sulphur in times which are defined by experiments. In this manner, particularly in the case of viscose silk, very different color or luster effects may be attained 10 even in undyed condition when the silk has been woven and eventually treated in accordance with this invention. Another mode of operating, particularly applicable to viscose silk, consists in producing a difference 15 of sulphur content in different parts of the same fibers by a mildly acting desulphuring agent e. g. a cold 1%  $Na_2S$  solution for a short time so that only the sulphur adhering to the surface of the fiber is removed, 20 while that contained in the core of the fiber remains. On subsequently dyeing according to this invention for instance with a 1% solution of  $AgNO_3$  with a sufficient quantity of sodium sulphite there is obtained a 25 lustrous brown black by  $Ag_2S$  colored fiber; on the other hand, it is also possible to dye only the outer surface of the sulphured fiber and subsequently to remove the sulphur from the core or to leave it in the core. 30 There is then obtained a colored fiber which is dull.

It is not necessary to bring about the difference in sulphur content of the fibers before the latter are made up into fabric 35 or the like; the process may be applied to a fabric made up of uniformly sulphured fibers. Thus it is possible to vary the sulphur content at particular places in such a fabric, for example the threads at a particular place in a woven fabric may be more or less freed from sulphur. In a fabric 40 treated in this manner the desired difference of color and luster can be produced by subsequent treatment according to this invention. The local reduction or removal of sulphur in a fabric is possible in several ways. For instance a pattern may be printed upon the fabric by means of a liquid or 45 paste which dissolves sulphur or combines with sulphur and after the fabric has been washed it may be treated in a dye-bath. For this purpose a 10 to 15% solution of  $Na_2S$ , thickened by any means of thickening, and the action of which may be supported by 50 heat, e. g. by steam, may be used. It is also possible to print upon the fabric a substance which repels water, such as wax, so as to protect the sulphur locally from solution and then to remove the sulphur from parts 55 not printed by means of a solvent.

Particularly in the case of viscose silk, the foregoing process results in producing very beautiful lustrous effects because the parts of the fabric which contain sulphur retain their dull appearance. In this manner there

are obtained the same effects as are produced by weaving a pattern of sulphured and non-sulphured threads in a Jacquard pattern loom. Obviously a suitable dyestuff may be printed together with a sulphur fixing or 70 sulphur dissolving liquid.

What I claim is:

1. A process of producing different exterior effects on textile fibers, yarns, webs or the like, consisting in creating a difference in the sulphur content of part of the fibers from the remaining part, said difference ranging between a small percentage and 100% of the sulphur content of the sulphur-containing material. 80

2. A process of producing different exterior effects on textile fibers, yarns, webs or the like, consisting in creating a difference in the sulphur content of part of the fibers from the remaining part, and thereafter 85 treating both parts in the same bath of a dye which does not cause dispersion of the sulphur in the bath.

3. A process of producing different exterior effects on textile fibers, yarns, webs or the like, which consists in giving to one part of the fibers a sulphur content different from that of another part, and thereafter 90 treating both parts in the same bath of a dye which is affected by the sulphur without causing dispersion of the sulphur in the 95 bath.

4. A process of producing different exterior effects on sulphur-containing textile fibers, yarns, webs or the like, which consists in treating part of the fibers with a mildly-acting desulphuring agent, so as to desulphur solely the outer surface of the treated fibers and thereby obtain a difference in the sulphur content of the fibers. 100

5. A process of producing different exterior effects on sulphur-containing textile fibers, yarns, webs or the like, which consists in treating part of the fibers with a mildly-acting desulphuring agent, so as to desulphur solely the outer surface of the treated fibers and thereby obtain a difference in the sulphur content of the fibers, and thereafter 110 treating all the fibers in the same bath of a dye which does not cause dispersion of the sulphur in the bath. 115

6. A process according to claim 5, in which the outer surface of the fibers is dyed by a dyestuff solution which is affected by the sulphur, and the core of the fibers is 120 subsequently desulphured.

7. A process of producing different exterior effects on textile fibers, yarns, webs or the like, which consists in creating a difference in the sulphur content of the fibers, and treating the fibers with a coloring agent which is affected by the sulphur to produce a difference of color between the more sulphured and less-sulphured parts. 125

8. A process according to claim 7, in

which the coloring agent is a metal salt solution which forms an insoluble metal compound with the sulphur of the fibers.

9. A process of producing different exterior effects on textile fibers, yarns, webs, or the like, which consists in creating a difference in the sulphur content of the fibers, treating such fibers with a metal salt solution which produces an insoluble metal com-

pound with the sulphur of the fibers, and 10 then dyeing with an organic dyestuff whereby the metal compound precipitated on the more sulphured fibers serves as a mordant so as to produce a difference of color from that produced on the less-sulphured fibers. 15

In testimony whereof I affix my signature.

HENDRIK JAN JAKOB JANSSEN.